

## UNITED STATES PATENT OFFICE.

CARLETON ELLIS, OF MONTCLAIR, NEW JERSEY, ASSIGNOR TO CHADELOID CHEMICAL COMPANY, A CORPORATION OF WEST VIRGINIA.

## PAINT AND VARNISH REMOVER.

No Drawing.

Application filed April 2, 1921. Serial No. 458,051.

*To all whom it may concern:*

Be it known that I, CARLETON ELLIS, a citizen of the United States, residing in the city of Montclair, State of New Jersey, have 5 invented certain new and useful Improvements in Paint and Varnish Removers, which is set forth in the following specification.

This invention relates to a composition adapted for use as a paint and varnish 10 mover and relates especially to a composition having a relatively high flashpoint and being of a substantially non-inflammable character or of such a low degree of inflammability that the composition may be 15 used safely even in the neighborhood of a flame.

*Benzol-acetone removers.*—The paint and varnish removers commonly used at the present time are made up of benzol, acetone and 20 wax and have highly inflammable properties. If a large surface coated with such a remover is accidentally ignited a dangerous fire may 25 ensue. The powerful action of a mixture of benzol and acetone has however established a standard of efficiency and rapidity of softening of paint and varnish which is difficult to approach by any other combination of 30 commercial solvents.

*Penetrating and loosening action.*—A 35 paint and varnish remover should have a powerful penetrating and loosening action on dried coats of paint or varnish and should not dry out quickly, allowing time for the removal of the softened paint by means of 40 a brush or putty knife or in other ways. Such a solvent must be capable of general use, that is must have a removing action on all kinds of paint and varnish so that one grade of remover will serve the painter in 45 all his operations of this character. Almost without exception the best removing effects are secured by light highly volatile solvents, these have not only a better penetrating action but seemingly soften the surface and convert it into a jelly-like material which is 50 readily removed. On the other hand heavy solvents which are much less volatile as a general rule have little penetrating power and action being quite sluggish in most cases 55 and not usually being capable of softening

the varnish to a jelly like easily removable film. In preparing a non-inflammable paint and varnish remover, which, other than its non-inflammability, has characteristics in common with the benzol acetone removers 55 mentioned above is difficult as the number of solvents available commercially which may be used in such composition is relatively limited if heavy solvents are excluded.

*Non-inflammability.*—The use of the term 60 non-inflammable as referred to herein does not mean necessarily that the composition cannot be ignited under severe test conditions but that it does not ignite readily so that an entire surface coated with the 65 remover will burst into flame on the application of a match. What is particularly meant by the term as used herein is that the composition in question when spread out on a 70 surface and the flame of a match applied 75 will not burst into instant ignition but in some cases may be ignited locally by superheating the surface through a prolonged application of the flame. Or if the surface is roughened and rolled up as for example by 75 running a putty knife through the softened mass and a lighted match is brought in contact with a projection of the varnish film this may burn slowly for a time and then the 80 flame will go out or it may even spread 80 slowly and gradually as the surface becomes heated. The rolled up varnish in this case probably acts to some extent as a wick. On the other hand the composition may have a 85 higher degree of non-inflammability such that on contact with a flame no flash or ignition of any kind occurs the flame of the match being extinguished when lighted end is pressed down into the liquid. Intermediate 90 these two is a grade which cannot be ignited when the remover is poured out on a flat surface and touched with a lighted match but on a vertical surface and by slight superheating ignition may be started and will travel upwardly along the vertical layer 95 of remover.

*Film formation.*—In order to use a volatile solvent or mixture of volatile solvents effectively it is necessary to have a retarder of evaporation. Paraffin wax is best for 100

this purpose, the hardest wax being most suitable. The wax forms a skin over the surface of the volatile solvents so that evaporation is very greatly reduced in amount 5 and will allow the solvents to perform their softening action. The manner in which a waxy film forms depends upon the amount of wax and the nature of the solvent. If a high proportion of a wax solvent is present 10 too great a quantity of wax will be dissolved thereby diluting the remover with inert material and reducing the amount of actual solvent material available.

*Odor.*—Painters are accustomed to work 15 with certain paint and varnish solvents such as turpentine, naphtha, gasoline and alcohol and do not take kindly to solvents which have odor which differ very greatly from these. It is important in a commercial article 20 to have the preparation possess an odor agreeable to the painter or at least one which he will not object to to such an extent as to refuse to employ the product. It is also desirable that the remover be free from any 25 highly objectionable odor such that when used, for example, in apartment houses the odor does not penetrate through the hallways to different apartments and cause complaint.

*Corrosive action.*—A composition which 30 has a corrosive action on the skin or which would stain the wood or raise the grain of the latter or which would corrode the tin cans ordinarily used as containers for products of this description is objectionable.

*Consistency.*—The consistency of the remover should, as far as possible, remain constant with the changes in temperature and not become a dense solid mass in the cold 40 and a thin rapidly evaporating liquid at higher climatic temperatures.

*Availability of raw material.*—The raw materials employed should be commercially available and should be fairly low in price as the cost of removing paint and varnish 45 by such solvent material must not exceed that of the old methods of scraping or burning off.

In the type of remover embodied in the present invention light volatile solvents are 50 made the basis of the composition, although the addition of heavy solvents is not precluded and these light volatile solvents preferably comprise a non-inflammable chlorinated hydrocarbon preferably trichlorethylene, 55 although tetrachlorethane or acetylene tetrachloride, carbon tetrachloride etc. may also be used in some cases. Carbon tetrachloride, generally speaking, is not recommended in compositions containing water on 60 account of the decomposition of the tetrachloride in the presence of moisture causing an acid reaction and if the composition is in a tin can the latter will be attacked and leakage results. Trichlorethylene is much 65 less likely to become acid and has a pleas-

anter odor than for example acetylene tetrachloride. The composition has a high flashpoint or degree of non-inflammability such that it is safe to use in the neighborhood of a flame and cannot be ignited by 70 sparks, lighted cigarettes etc. A good degree of film formation with not an excessive amount of wax is obtained. The odor while noticeable is not of a disagreeable nature and after the operator has used the composition 75 for a time the odor will be found unobjectionable to most persons.

A formula affording a composition having fair softening and penetrating qualities coupled with a not unpleasant odor is made 80 by mixing 60 parts by volume of trichlorethylene, 25 parts of ethyl acetate and 15 parts of monochlorbenzol. To this is added from 7 to 15 per cent of hard paraffin wax. The proportion of trichlorethylene in this 85 composition is considerable and being a pronounced wax solvent a somewhat larger proportion of wax is used than in some of the following compositions. Trichlorethylene does not have quite as strong an inflammability suppressing power as carbon tetrachloride, but, as stated, it is more desirable 90 on account of odor and comparative freedom from action on metal surfaces. The inflammability suppressing power is dependent to 95 a considerable extent on the vapor tension of the solvent and is more or less correlated with the boiling point. For example acetone boiling at 56° C. is not so suitable for use 100 in the present composition because it takes in the neighborhood of 90 volumes of trichlorethylene to 10 volumes of acetone to sufficiently repress the inflammability of the latter. Thus such a composition would not 105 very well serve as a paint and varnish remover because there would be an insufficient amount of softening agent, namely the acetone and such a high proportion of wax solvent that excessive amounts of wax would have to be employed. On the other hand 110 when the boiling point is above 75° C. and preferably above 80° C. a more substantial amount of the softening agent may be 115 utilized. Thus in the case of ethyl acetate boiling at 77° C. in the neighborhood of 25 per cent may be used and the same is true of methyl ethyl ketone boiling at 79° C. Such mixtures are difficult to ignite with a flame and the combustion as a rule does not continue or spread from the superheated portion 120 at the place of ignition.

The addition of heavy solvents in small quantity up to 30% or more in some cases improves the degree of non-inflammability and aids in keeping the composition moist 125 over a considerable period of time so that for example a surface to which remover has been applied in the afternoon will keep moist over night so that the finish may be removed on the following morning. Exam- 130

5 ples of heavy solvents or solvents which are relatively heavy in comparison with some of the light penetrating solvent material preferably employed, are compounds such

5 as aniline, toluidine, xylidine, phenol or car-  
bolic acid, cresol and cresylic acid and higher phenols. Also what is commercially known as tar acids and is usually a mixture of cresols and higher phenols but does not 10 contain phenol itself. The dichlorbenzols are heavy non-inflammable bodies, the paradichlorbenzol being solid while the ortho compound is liquid. The latter is preferable for solvent purposes. Among other 15 solid solvents may be mentioned camphor. Fusel oil and also refined amyl alcohol, amyl acetate and other amyl esters such as amyl lactate may be used in some cases. Butyl alcohol is not so heavy a solvent but its 20 odor and also the odor of fusel oil and amyl alcohol is usually objectionable if the amount present is substantial. Propyl alcohol and isopropyl alcohol stand intermediate the heavy solvents and the light solvents. Ani- 25 sol, phenetol and chlorhydrins also may be noted as heavier solvents for addition to compositions such as indicated above.

For example referring to the composition made by mixing 60 parts by volume of 30 trichlorethylene, 25 volumes of ethyl acetate and 15 parts of monochlorbenzol with sufficient wax to exert the desired film forming action the following compositions were made. To 8 parts by volume of the stock 35 solution, 2 parts of aniline were introduced. This did not materially change the inflammability but the composition acted as a fairly efficient remover. In another case 9 parts of stock solution were mixed with 1 40 part of tar acids. In another case 8 parts of the stock solution were mixed with 2 parts of tar acids, the mixture had better non-inflammable qualities than in the case where aniline was used. In another case 1 part 45 and 2 parts of paradichlorbenzol were added to 9 parts and 8 parts respectively of the stock solution. This mixture catches fire on applying a flame but goes out as soon as the flame is removed, the combustion does 50 not spread. Removers also were made by adding 1 part of anisol and also 1 part of phenetol to the stock solution. The phenetol composition appears to be slightly more difficult at ignition than that containing anisol. An excellent sufficiently non-inflammable 55 remover was made from 9 parts of stock solution and 1 part of anhydrous chlorhydrins, these being a mixture of ethylene and propylene chlorhydrins. 7 volumes of the 60 stock solution and 3 volumes of anhydrous chlorhydrin gave a remover of an improved degree of non-inflammability.

In connection with the matter of proportioning the amount of non-inflammable sol- 65 vent to a penetrating or loosening volatile

inflammable solvent the following may be noted with respect to ethyl acetate:

Ethyl acetate with acetylene tetrachloride—

20% flashes and burns. 70  
30% flashes and burns.  
40% flashes but not so readily.  
50% does not flash but will burn.  
60% ignites.  
70% will not ignite. 75

The criticism of a composition made up of 30% ethyl acetate and 70% acetylene tetrachloride is that the odor of the latter in such a predominating amount is objectionable and as acetylene tetrachloride is fairly costly on a volume basis the composition is expensive. Also 70% of acetylene tetrachloride is likely to exert too great a solvent action on wax so that a large proportion of the latter is required. 85

Ethyl acetate with carbon tetrachloride—  
30% flashes and burns.

40% ignites and burns with a smoky flame.  
50% will not ignite. 85

While only 50% of carbon tetrachloride is used in this case showing that the latter is more powerful in suppressing inflammability than acetylene tetrachloride it should be noted that carbon tetrachloride rather readily turns acid and attacks metal containers. 95

Isopropyl alcohol with acetylene tetrachloride—

30% flashes and burns.  
40% ignites readily. 100  
50% ignites but less readily.  
60% will just ignite.  
65% will not ignite.

Isopropyl alcohol with carbon tetrachloride—  
20% ignites. 105  
30% will not ignite.

In order to determine whether paradichlorbenzol would result in raising the flash-point of these mixtures a mixture of 50% ethyl acetate, 50% acetylene tetrachloride was saturated with paradichlorbenzol (60 to 70% of the weight of the solvent), this was found to burn just as readily as before the addition of the paradichlorbenzol. A mixture of 60% ethyl acetate, 40% carbon tetrachloride was saturated with paradichlorbenzol (about 80% of the weight of the solvent), this was found to burn equally as readily as before the addition of dichlorbenzol. 110 115 120

Orthodichlorbenzol as stated is a liquid and is non-inflammable and combustible with great difficulty. When mixed with benzyl alcohol which also is very difficult to ignite a mixture is obtained which may be used as a paint and varnish remover and which is practically free from any criticism of inflammability. Owing to the slow evaporating properties of these solvents the addition of 125 130

wax is not necessary in many cases. Such a remover, however, is so slow in its action that it does not give commercially satisfactory results as a rule. If a composition such as is now generally used for paint and varnish removing purposes consisting of benzol and acetone or alcohol with wax be taken as a standard for comparison, e. g. a mixture of equal parts by volume of benzol and methyl acetone with which is incorporated 5% of paraffin wax, the speed of softening paint or varnish may be represented by the figure 1. While in the case of the mixture of orthodichlorbenzol and benzyl alcohol the figure will be from 3 to 5, denoting that 3 to 5 times as long a period is required to remove the same coating of paint or varnish as is requisite with the standard benzol-acetone remover. The addition of ethyl 10 alcohol or better methyl ethyl ketone or ethyl acetate materially increases the speed of the above mentioned benzyl alcohol composition but makes the latter readily inflammable. A volatile chlorinated solvent may 15 therefore be added proportionate in amount to the amount of volatile inflammable solvent. From the foregoing it will be noted that certain ratios of carbon tetrachloride, acetylene tetrachloride or trichlorethylene to 20 other volatile inflammable solvents are required to suppress the inflammability of the latter. This ratio should be substantially 25 preserved in the presence of heavy solvents such as benzyl alcohol or orthodichlorbenzol 30 as the effect of the latter on reducing the inflammability of the higher volatile solvent is small. Of the heavy solvents phenol and cresol appear to have the greatest effect but 35 this is not sufficiently high in view of the 40 relatively small proportion of such carbolic acid material as may be ordinarily used in a remover to permit of the use of phenol or cresol as deterrents of inflammability, at least to any material extent. Reliance must 45 be had in such cases on non-inflammable solvents of a volatile nature such as the chlorinated compounds referred to above.

Orthodichlorbenzol is a substantially less inflammable vehicle than the monochlorbenzol. While the latter is ignited after a flame 50 has been held for only a short time in contact with a horizontal surface moistened with the latter solvent it is quite difficult under these conditions to ignite the dichlor compound.

A composition made with 50% by volume 55 of trichlorethylene, 25% of benzyl alcohol and 25% of ethyl alcohol with approximately 5% of paraffin wax while a fairly safe remover to use is nevertheless ignited after a short application of a flame. On 60 reducing the ethyl alcohol to 20% and increasing the benzyl alcohol to 30% a composition is obtained which has a sufficiently 65 high flashpoint to be of general utility.

Ethyl alcohol is however not as good a solvent for paint and varnish as ethyl acetate or methyl ethyl ketone which have boiling points in the neighborhood of that of ethyl alcohol. If ethyl acetate is substituted for ethyl alcohol so that the liquid vehicle in the composition is approximately 50% of trichlorethylene, 30% benzyl alcohol and 20% ethyl acetate, with which is incorporated from 4 to 6% of paraffin wax, a 70 highly efficient paint and varnish remover is obtained which in comparison with the standard inflammable type of benzol-acetone remover has a speed rating of between 1 and 1.5, thus this composition while safe 75 to use has the speed requisite for commercial application. It does not contain any undue amount of wax so that useful solvent material is not displaced by non-solvent wax and the odor is not disagreeable. When the 80 composition is modified to 10% ethyl acetate, 30% benzyl alcohol and 60% of trichlorethylene, with approximately the same amount of wax, a very safe composition is secured which is practically incombustible. It is extremely difficult to ignite such a 85 composition when applied to a painted surface and even on boiling the composition the vapors do not burn violently, nor do they set fire to the liquid itself. Thus a 90 composition containing trichlorethylene or similar chlorinated solvent in excess, a lesser amount of a heavier solvent such as benzyl alcohol or diacetone alcohol or chlorhydrin or mixtures of such heavy solvents and a 95 still smaller amount of an inflammable volatile solvent, preferably boiling between 75° C. and 100° C., as for example ethyl alcohol, ethyl acetate, methyl ethyl ketone, propyl 100 or isopropyl alcohol may be employed in 105 making suitable paint and varnish removing compositions of the requisite degree of non-inflammability and especially in the case of compositions containing ethyl acetate or methyl ethyl ketone also possessing a rate 110 of softening or removing action comparable with standard inflammable remover as aforesaid.

Solvent naphtha may be used as an extending 115 medium in some cases but it is not a very effective solvent and ordinarily is not recommended for an active remover, its principal utility is as a cheapening and bulking agent. Propyl or isopropyl acetate or other esters may be employed in some 120 cases. On the other hand isopropyl ether is not recommended for non-inflammable compositions as it has too low a flashpoint. In this respect it is like acetone or methyl alcohol, the presence of which to the extent 125 of 5% or so is very quickly indicated by the lowering of the flashpoint of the composition necessitating increased amounts of a more costly non-inflammable solvent such as acetylene tetrachloride or trichlorethyl- 130

ene. As indicated above, too large a proportion of a hydrocarbon solvent or chlorinated solvent having a strong solvent action on wax throws the composition out of balance and the removing action is not as effective as when more of compounds of a generally alcoholic nature are present; this including not only the alcohols themselves but esters, ketones and the like which have a generally precipitating or non-solvent action on waxy material.

The addition of selenium oxychloride to the above compositions is not precluded and this material has considerable solvent action on paint and varnish, however its generally acid nature makes it ordinarily undesirable, it being one object, in the preferred form of the present invention, to produce a removing composition of a substantially neutral character which will not injure the wood or the hands of the users, destroy paint brushes or corrode the metal containers.

In a number of useful formulæ made in accordance with the present invention and involving a heavy solvent in conjunction with readily volatile solvents, as for example benzyl alcohol as a heavy solvent, ethyl alcohol or ethyl acetate as a volatile inflammable solvent, and trichlorethylene as a volatile non-inflammable solvent, the proportion of the trichlorethylene may be approximately 2½ times that of the volatile alcoholic solvent.

The exact proportions however required to meet the requisite degree of non-inflammability vary to some extent with the general character of the solvents employed, as for example 50 parts by volume of trichlorethylene, 30 parts of diacetone alcohol and 20 parts of ethyl acetate may be ignited on continued application of a flame, while 60 parts of trichlorethylene, 30 parts diacetone alcohol and 10 parts of ethyl acetate is not readily inflammable.

45 50 parts of trichlorethylene, 30 parts of orthodichlorbenzol and 20 parts of ethyl acetate is more readily ignited.

Among the waxes which may be employed to advantage in the above composition, in order to prevent or minimize evaporation, are paraffin and ceresin wax. The former is better for liquid remover while the latter in sufficient proportion gives a pasty remover of smooth consistency. Other 50 waxes such as beeswax, carnauba, montan, candelila wax and the like may be added to the foregoing waxes or used by themselves but are not as satisfactory as paraffin wax. Thickening agents such as soaps, 55 nitrocellulose, cellulose acetate and the like 60 may also be used in some cases.

What I claim is:—

1. A paint and varnish removing composition adapted for softening dried films of paint and varnish which comprises a

70 mixture of solvents including a volatile inflammable solvent and a volatile non-inflammable solvent, comprising trichlorethylene, the proportion of said non-inflammable solvent being sufficient to suppress the inflammability of the former so that the composition when contacted with a flame does not readily ignite and propagate a dangerous combustion; the composition containing wax sufficient in amount to serve 75 as an efficient evaporation-retarding substance for the volatile solvents but said wax not being sufficient in quantity to displace a material amount of the volatile solvents; said composition being capable of softening dried coats of paint and varnish at a rate 80 not materially slower than inflammable paint and varnish remover made from equal volumes of benzol and acetone with about 85 5% of wax.

2. A paint and varnish removing composition adapted for softening dried films of paint and varnish which comprises a mixture of solvents including a volatile inflammable solvent and major proportion of a volatile non-inflammable solvent comprising trichlorethylene, the proportion of said non-inflammable solvent being sufficient to suppress the inflammability of the former so that the composition when contacted with a flame does not readily ignite and propagate the combustion; the composition containing wax sufficient in amount to serve 90 as an efficient evaporation-retarding substance for the volatile solvents but said wax not being sufficient in quantity to displace a material amount of the volatile solvents; said composition being capable of softening dried coats of paint and varnish at a rate 95 not materially slower than inflammable paint and varnish made from equal volumes of benzol and acetone with about 5% of wax.

3. A paint and varnish removing composition adapted for softening dried films of paint and varnish which comprises a 100 mixture of solvents including a volatile inflammable solvent boiling between 75° and 100° C., and a volatile non-inflammable solvent comprising trichlorethylene, the proportion of said non-inflammable solvent 105 being sufficient to suppress the inflammability of the former so that the composition when contacted with a flame does not readily ignite and propagate the combustion; the composition containing wax sufficient 110 in amount to serve as an efficient evaporation retarding substance for the volatile solvents but said wax not being sufficient in quantity to displace a material amount of the volatile solvents; said composition 115 being capable of softening dried coats of paint and varnish at a rate not materially slower than inflammable paint and varnish remover made from equal volumes of benzol and acetone with about 5% of wax.

4. A paint and varnish removing composition adapted for softening dried films of paint and varnish which comprises a mixture of solvents including a heavy solvent, 5 a volatile inflammable solvent boiling under 100° C., and at least an equal proportion of a volatile non-inflammable solvent, the proportion of the latter being sufficient to suppress the inflammability of the former so that the composition when contacted with a flame does not readily ignite and propagate the combustion; the composition containing wax sufficient in amount 10 to serve as an efficient evaporation retarding substance for the volatile solvents but said wax not being sufficient in quantity to displace a material amount of the volatile solvents; said composition being capable of softening dried coats of paint and varnish 15 at a rate at least two-thirds as rapidly as inflammable paint and varnish remover 20 made from equal volumes of benzol and acetone with about 5% of wax.
5. A paint and varnish remover comprising wax, trichlorethylene, diacetone alcohol 25 and ethyl acetate.
6. A paint and varnish remover consisting of wax, trichlorethylene, an alcohol and a volatile solvent whose boiling point is above 75° C. and not exceeding 100° C. 30
7. A paint and varnish remover consisting of wax, trichlorethylene, a heavy alcohol and an ester whose boiling point is above 75° C. and not exceeding 100° C.
8. A paint and varnish remover comprising wax, trichlorethylene, diacetone alcohol and a volatile alcoholic solvent whose boiling point is above 75° C. and not exceeding 100° C. 35

In testimony whereof, I have signed this 40 specification.

CARLETON ELLIS.